# EUROPEAN PATENT SPECIFICATION

(11) **EP 1 049 818 B1**
(45) Date of publication and mention of the grant of the patent: **29.12.2004**
(21) Application number: 99900110.0
(22) Date of filing: 19.01.1999
(51) Int. Cl.: C25C 3/12, C25C 7/02

(54) **NON-CARBON METAL-BASED ANODES FOR ALUMINIUM PRODUCTION CELLS**
KOHLENSTOFF-FREIE ANODEN AUF BASIS VON METALLEN FÜR ALUMINIUM-ELEKTROGEWINNUNGSZELLEN
ANODES METALLIQUES EXEMPTES DE CARBONE POUR CELLULES DE PRODUCTION D'ALUMINIUM

(30) Priority: 20.01.1998 WO PCT/IB98/00080; 30.07.1998 US 126206; 30.07.1998 US 126840; 30.07.1998 US 126359
(43) Date of publication of application: 08.11.2000
(73) Proprietor: MOLTECH Invent S.A., 1520 Luxembourg (LU)
(72) Inventor: DE NORA, Vittorio, Nassau (BS); DURUZ, Jean-Jacques, CH-1204 Geneva (CH)
(74) Representative: Cronin, Brian
(86) International application number: PCT/IB1999/000084
(87) International publication number: WO 1999/036594

(56) References cited:
- EP-A- 0 306 101
- WO-A-93/20026
- US-A- 4 541 912

## Description

### Field of the Invention

This invention relates to non-carbon metal-based anodes for use in cells for the electrowinning of aluminium by the electrolysis of alumina dissolved in a molten fluoride-containing electrolyte, and to methods for their fabrication and reconditioning, as well as to electrowinning cells containing such anodes and their use to produce aluminium.

### Background Art

The technology for the production of aluminium by the electrolysis of alumina, dissolved in molten cryolite containing salts, at temperatures around 950°C is more than one hundred years old.

This process, conceived almost simultaneously by Hall and Héroult, has not evolved as many other electrochemical processes.

The anodes are still made of carbonaceous material and must be replaced every few weeks. The operating temperature is still not less than 950°C in order to have a sufficiently high solubility and rate of dissolution of alumina and high electrical conductivity of the bath.

The anodes have a very short life because during electrolysis the oxygen which should evolve on the anode surface combines with the carbon to form polluting CO₂ and small amounts of CO and fluoride-containing dangerous gases. The actual consumption of the anode is as much as 450 Kg/Ton of aluminium produced which is more than 1/3 higher than the theoretical amount of 333 Kg/Ton

The frequent substitution of the anodes in the cells is still a clumsy and unpleasant operation. This cannot be avoided or greatly improved due to the size and weight of the anode and the high temperature of operation.

Several improvements were made in order to increase the lifetime of the anodes of aluminium electrowinning cells, usually by improving their resistance to chemical attacks by the cell environment and air to those parts of the anodes which remain outside the bath. However, most attempts to increase the chemical resistance of anodes were coupled with a degradation of their electrical conductivity.

US Patent 4,614,569 (Duruz/Derivaz/Debely/Adorian) describes non-carbon anodes for aluminium electrowinning coated with a protective coating of cerium oxyfluoride, formed in-situ in the cell or pre-applied, this coating being maintained by the addition of cerium compounds to the molten cryolite electrolyte. This made it possible to have a protection of the surface only from the electrolyte attack and to a certain extent from the gaseous oxygen but not from the nascent monoatomic oxygen.

EP Patent application 0 306 100 (Nyguen/Lazouni/Doan) describes anodes composed of a chromium, nickel, cobalt and/or iron based substrate covered with an oxygen barrier layer and a ceramic coating of nickel, copper and/or manganese oxide which may be further covered with an in-situ formed protective cerium oxyfluoride layer.

Likewise, US Patents 5,069,771, 4,960,494 and 4,956,068 (all Nyguen/Lazouni/Doan) disclose aluminium production anodes with an oxidized copper-nickel surface on an alloy substrate with a protective barrier layer. However, full protection of the alloy substrate was difficult to achieve.

A significant improvement was described in US Patent 5,510,008, and in International Application WO96/12833 (Sekhar/Liu/Duruz) involved a anode having a micropyretically produced body from a combination of nickel, aluminium, iron and copper and oxidising the surface before use or in-situ during electrolysis. By said micropyretic methods materials have been obtained whose surfaces when oxidised are active for the anodic reaction and whose metallic interior has low electrical resistivity to carry a current from high electrical resistant surface to the busbars. However it would be useful, if it were possible, to simplify the manufacturing process of these materials obtained from powders and increase their life to make their use economic.

Metal or metal based anodes are highly desirable in aluminium electrowinning cells instead of carbon-based anodes. Many attempts were made to use metal-based anodes for aluminium production, however they were never adopted by the aluminium industry because of their poor performance.

### Objects of the Invention

An object of the invention is to substantially reduce the consumption of the active anode surface of an aluminium electrowinning anode which is attacked by the nascent oxygen by enhancing the reaction of nascent oxygen to biatomic molecular gaseous oxygen.

Another object of the invention is to provide a coating for an aluminium electrowinning anode which has a high electrochemical activity and also a long life and which can be replaced as soon as such activity decreases or when the coating is worn out.

A major object of the invention is to provide an aluminium electrowinning anode which has no carbon so as to eliminate carbon-generated pollution and reduce the cost of operation.

### Summary of the Invention

The invention provides a non-carbon metal-based anode of a cell for the electrowinning of aluminium, in particular by the electrolysis of alumina dissolved in a molten fluoride-containing electrolyte. The anode comprises an electrically conductive metal substrate resistant to high temperature, the surface of which becomes passive and substantially inert to the electrolyte, and an electrochemically active coating adherent to the surface of the metal substrate making and keeping the surface of the anode conductive and electrochemically active for the oxidation of oxygen ions present at the electrolyte interface.

Whereas conventional coatings are usually used to protect a conductive substrate of a cell component from chemical and/or mechanical attacks destroying the substrate, this particular treatment is applied in the form of a coating onto a passivatable substrate to maintain the anode surface conductive and electrochemically active and protect it from electrolyte attack wherever the coating covers the surface even though the coating may be imperfect or incomplete.

This allows the coated surfaces of the anode to remain electrochemically active during electrolysis, while the remaining parts of the surface of the metal substrate become inert to the electrolyte. This passivation property offers a self-healing effect, i.e. when the surface of the anode is imperfectly covered, damaged or partly worn out, parts of the metal substrate which come into contact with the electrolyte are automatically passivated during electrolysis and become inert to the electrolyte and not corroded.

Metal substrates providing for this self-healing effect in molten fluoride-based electrolyte may be made of one or more metals selected from nickel, cobalt, chromium, molybdenum, tantalum and the Lanthanide series of the Periodic Table, and their alloys or intermetallics, such as nickel-plated copper.

The coatings usually comprise:
a) at least one electrically conductive and electrochemically active constituent,
b) an electrocatalyst, and
c) a bonding material substantially resistant to cryolite and oxygen for bonding these constituents together and onto the passivatable metal substrate.

These constituents are usually co-applied though it is possible to provide sequential application of the different constituents.

The presence of one or more electrocatalysts is desirable, although not essential for the invention. Likewise the presence of bonding material is not always necessary.

Coatings can be obtained by applying their active constituents and their precursors by various methods which can be different for each constituent and can be repeated in several layers. For example, a coating can be obtained by directly applying a powder onto the passivatable metal substrate or constituents of the coating may be applied from a slurry or suspension containing colloidal or polymeric material. The colloidal material can be a binder solely or can be part of the active material. The colloidal material may include at least one colloid selected from colloidal alumina, ceria, lithia, magnesia, silica, thoria, yttria, zirconia, tin oxide, zinc oxide and colloid containing the active material.

When a slurry or a suspension containing colloidal material is applied the dry colloid content corresponds to up to 50 weight% of the colloid plus liquid carrier, usually from 10 to 20 weight%.

The coating can be applied on the substrate by plasma spraying, physical vapor deposition (PVD), chemical vapor deposition (CVD), electrodeposition or callendering rollers. A slurry or a dispersion is preferably applied by rollers, brush or spraying.

Usually the electrochemically active constituent(s) is/are selected from oxides, oxyfluorides, phosphides, carbides and combinations thereof.

The oxide may be present in the electrochemically active layer as such, or in a multi-compound mixed oxide and/or in a solid solution of oxides. The oxide may be in the form of a simple, double and/or multiple oxide, and/or in the form of a stoichiometric or non-stoichiometric oxide.

The oxides may be in the form of spinels and/or perovskites, in particular spinels which are doped, non-stoichiometric and/or partially substituted. Doped spinels may comprise dopants selected from Ti⁴⁺, Zr⁴⁺, Sn⁴⁺, Fe⁴⁺, Hf⁴⁺, Mn⁴⁺, Fe³⁺, Ni³⁺, Co³⁺, Mn³⁺, Al³⁺, Cr³⁺, Fe²⁺, Ni²⁺, Co²⁺, Mg²⁺, Mn²⁺, Cu²⁺, Zn²⁺ and Li⁺.

Such a spinel may be a ferrite, in particular a ferrite selected from cobalt, manganese, molybdenum, nickel and zinc, and mixtures thereof. The ferrite may be doped with at least one oxide selected from the group consisting of chromium, titanium, tantalum, tin, zinc and zirconium oxide.

Nickel-ferrite or nickel-ferrite based constituents are advantageously used for their resistance to electrolyte and may be present as such or partially substituted with Fe²⁺.

The coating may also contain a chromite which is usually selected from iron, cobalt, copper, manganese, beryllium, calcium, strontium, barium, magnesium, nickel and zinc chromite.

The electrochemically active constituents of the coating may be selected from iron, chromium, copper and nickel, and oxides, mixtures and compounds thereof, as well as a Lanthanide as an oxide or an oxyfluoride such as cerium oxyfluoride, and mixtures thereof.

When an electrocatalyst is present in the coating it is selected preferably from noble metals such as iridium, palladium, platinum, rhodium, ruthenium, or silicon, tin and zinc, the Lanthanide series of the Periodic Table and mischmetal oxides, and mixtures and compounds thereof.

Coatings can be formed with or without reaction at low or high temperature. A reaction can either take place among the constituents of the coating; or between the constituents of the coating and the passivatable metal substrate. When no reaction takes place to form the coating the active constituents must already be present in the applied material, for example in a slurry or suspension applied onto the substrate.

In order to manufacture these anodes any electrically conductive and heat-resisting materials may be used. However, metals which do not offer the self-healing effect can only be used as metal cores which must be coated with a layer forming the passivatable metal substrate having this self-healing effect particularly when exposed to a fluoride-containing electrolyte, such as cryolite.

The metal core may comprise metals, alloys, intermetallics, cermets and conductive ceramics, such as metals selected from copper, chromium, cobalt, iron, aluminium, hafnium, molybdenum, nickel, niobium, silicon, tantalum, titanium, tungsten, vanadium, yttrium and zirconium, and combinations and compounds thereof.

For instance, the core may be made of an alloy comprising 10 to 30 weight% of chromium, 55 to 90 weight% of at least one of nickel, cobalt and/or iron and 0 to 15 weight% of at least one of aluminium, hafnium, molybdenum, niobium, silicon, tantalum, tungsten, vanadium, yttrium and zirconium.

The core may be covered with an oxygen barrier layer. This layer may be obtained by oxidising the surface of the core when it contains chromium and/or nickel or by applying a precursor of the oxygen barrier layer onto the core and heat treating. Usually, the oxygen barrier layer comprises chromium oxide and/or black non-stoichiometric nickel oxide.

The oxygen barrier layer may be covered in turn with at least one protective layer consisting of copper or copper and at least one of nickel and cobalt, and/or (an) oxide(s) thereof to protect the oxygen barrier layer by inhibiting its dissolution into the electrolyte. For instance, the oxygen barrier layer may be coated first with a nickel layer and then with a copper layer, heat treated for several hours in an inert atmosphere, such as 5 hours at 1000°C in argon, to interdiffuse the nickel and the copper layer, and upon heat treatment in an oxidising media, such as an air oxidation for 24 hours at 1000°C, the interdiffused and oxidised nickel-copper layer constitutes a good a protective layer.

The invention relates also to a method of manufacturing the described non-carbon metal-based anode. The method comprises coating a substrate of electrically conductive metal resistant to high temperature the surface of which during electrolysis becomes passive and substantially inert to the electrolyte with at least one layer containing electrochemically active constituents or precursors thereof and heat-treating the or each layer on the substrate to obtain a coating adherent to the metal substrate making the surface of the anode electrochemically active for the oxidation of oxygen ions present at the electrolyte interface.

The method of the invention can be applied for reconditioning the non-carbon metal-based anode when at least part of the active coating has been dissolved or rendered non-active or dissolved. The method comprises clearing the surface of the substrate before re-coating said surface with a coating adherent to the passivatable metal substrate once again making the surface of the anode electrochemically active for the oxidation of oxygen ions.

Another aspect of the invention is a cell for the production of aluminium by the electrolysis of alumina dissolved in a fluoride-containing electrolyte, in particular a fluoride-based electrolyte or a cryolite-based electrolyte or cryolite, having non-carbon metal-based anodes comprising an electrically conductive passivatable metal substrate and a conductive coating having an electrochemically active surface as described hereabove.

Preferably, the cell comprises at least one aluminium-wettable cathode. Even more preferably, the cell is in a drained configuration by having at least one drained cathode on which aluminium is produced and from which aluminium continuously drains.

The cell may be of monopolar, multi-monopolar or bipolar configuration. A bipolar cell may comprise the anodes as described above as a terminal anode or as the anode part of a bipolar electrode.

Preferably, the cell comprises means to improve the circulation of the electrolyte between the anodes and facing cathodes and/or means to facilitate dissolution of alumina in the electrolyte. Such means can for instance be provided by the geometry of the cell as described in co-pending application PCT/IB98/00161 (de Nora/Duruz) or by periodically moving the anodes as described in co-pending application PCT/IB98/00162 (Duruz/Bellò).

The cell may be operated with the electrolyte at conventional temperatures, such as 950 to 970°C, or at reduced temperatures as low as 750°C.

The invention also relates to the use of such an anode for the production of aluminium in a cell for the electrowinning of aluminium by the electrolysis of alumina dissolved in a fluoride-containing electrolyte, wherein oxygen ions in the electrolyte are oxidised and released as molecular oxygen by the electrochemically active anode coating.

The invention will now be described in the following examples.

### Example 1

An non-carbon metal-based anode is prepared according to the invention by hot calendar rolling at 900°C of nickel ferrite particles having a particle size of 10-50 micron into a nickel metal sheet of 2 mm thickness used as an electrically conductive substrate for the anode. The nickel ferrite particles are coated onto the nickel sheet in an amount of 500 g/m².

After coating, the anode was tested in an electrolytic cell using cryolite with 6 weight% alumina as an electrolyte and a carbon cathode covered with molten aluminium. The anode was polarised at 1 A/cm² for 93 hours and sustained this current density during the entire test, the cell voltage remaining comprised between 5.5 and 5.8 Volts.

At the end of the test, the anode was dimensionally unchanged and no sign of corrosion could be detected at the anode surface.

### Example 2

A non-carbon metal-based anode according to the invention was obtained from a nickel substrate which was coated with a slurry with subsequent heat-treatment.

The slurry was made from a solution consisting of 10 ml of colloidal magnesia acting as a binder mixed with 20 g of nickel ferrite powder providing the electrochemically active constituents, as described in Example 1.

The slurry was then applied onto the substrate by means of a brush. 15 successive layers were applied onto the substrate. Each time a layer had been applied onto the substrate, the layer was cured on the substrate by a heat treatment at 500°C for 15 minutes before applying the next layer.

After coating the substrate with the 15 successive layers the anode had a final coating of 0.6 to 1.0 mm thick.

The anode was then tested in a laboratory scale cell for the electrowinning of aluminium. 10 minutes after immersing the anode into the electrolytic bath the anode was extracted from the cell. The parts of the anodes which were not protected by the coating had been passivated under the effect of the current by the formation of an inert and adherent nickel oxide layer formed on the uncoated surfaces which could be observed by optical microscopy and scanning electron microscopy of a cross section of the anode after test.

### Example 3

Similarly to Example 2, a coating was applied onto a nickel substrate in 10 layers, except that 0.2 g of iridium powder acting as a catalyst were added to the mixture of colloidal alumina with nickel-nickel ferrite.

Similar results were observed.

## Claims

1. A method of manufacturing a non-carbon metal-based anode of a cell for the electrowinning of aluminium, in particular by the electrolysis of alumina dissolved in fluoride-containing electrolyte, said method comprising coating a substrate of electrically conductive metal resistant to high temperature and the surface of which becomes passive and substantially inert to the electrolyte with at least one layer of an electrochemically active coating precursor in the form of a slurry or suspension containing at least one electrochemically active constituent or a precursor thereof, and heat-treating the or each layer on the substrate to obtain a coating adherent to the passivatable metal substrate making the surface of the anode electrochemically active for the oxidation of oxygen ions present at the electrolyte interface.

2. The method of claim 1, wherein the passivatable metal substrate comprises at least one metal selected from nickel, cobalt, chromium, molybdenum, tantalum and the Lanthanide series, and their alloys or intermetallics.

3. The method of claim 1, wherein the coating is formed by further applying a bonding material substantially resistant to cryolite for bonding the constituents of the coating together and onto the passivatable metal substrate.

4. The method of claim 1, wherein the coating is obtained from a slurry or suspension containing colloidal or polymeric material, in particular at least one of alumina, ceria, lithia, magnesia, silica, thoria, yttria, zirconia, tin oxide and zinc oxide, and colloids containing active constituents of the coating or precursors thereof, all in the form of colloids or polymers.

5. The method of claim 1, comprising reacting constituents of the coating precursor among themselves to form the coating, or reacting at least one constituent of the coating precursor with the passivatable metal substrate to form the coating.

6. The method of claim 1, wherein the coating precursor is applied onto the substrate by rollers, brush or spraying.

7. The method of claim 1, comprising coating the passivatable metal substrate onto an electronically conductive core, and forming an oxygen barrier layer on the core in particular by oxidising the surface of the core to form the oxygen barrier layer, or by applying a precursor of the oxygen barrier layer onto the core and heat treating.

8. The method of claim 7, comprising covering the oxygen barrier layer with at least one protective layer consisting of copper or copper and at least one of nickel and cobalt, and/or oxides thereof to protect the oxygen barrier layer by inhibiting its dissolution into the electrolyte.

9. The method of claim 1 for reconditioning a non-carbon metal-based anode having a passivatable substrate with an electrochemically active coating, when at least part of the active coating has become non-active or worn out, said method comprising clearing the surface of the substrate before re-coating said surface with a coating applied from said slurry or suspension.

10. A non-carbon metal-based anode of a cell for the electrowinning of aluminium, in particular by the electrolysis of alumina dissolved in a molten fluoride-containing electrolyte, comprising an electrically conductive metal substrate resistant to high temperature, the surface of which becomes passive and substantially inert to the electrolyte, and an electrochemically active coating adherent to the surface of the metal substrate making and keeping the surface of the anode conductive and electrochemically active for the oxidation of oxygen ions present at the electrolyte interface, said coating containing electrochemically active constituents in a colloid obtainable from at least one electrochemically active constituent or a precursor thereof in a colloid-containing slurry or suspension.

11. The anode of claim 10, wherein the passivatable metal substrate comprises at least one metal selected from nickel, cobalt, chromium, molybdenum, tantalum and the Lanthanide series, and their alloys or intermetallics.

12. The anode of claim of claim 11, wherein the passivatable metal substrate is nickel-plated copper.

13. The anode of claim 10, wherein the coating further comprises at least one electrocatalyst or a precursor thereof for the formation of oxygen gas, in particular electrocatalyst(s) selected from iridium, palladium, platinum, rhodium, ruthenium, silicon, tin and zinc, the Lanthanide series and mischmetal, and their oxides, mixtures and compounds thereof.

14. The anode of claim 10, wherein the coating further comprises a bonding material substantially resistant to cryolite for bonding the constituents of the coating together and onto the passivatable metal substrate.

15. The anode of claim 10, wherein the coating is a heat-treated slurry or suspension containing at least one heat-treated colloid or polymer selected from heat-treated colloidal or polymeric alumina, ceria, lithia, magnesia, silica, thoria, yttria, zirconia, tin oxide, and zinc oxide, and colloids containing active constituents of the coating or precursors thereof, all in the form of heat treated colloids or polymers.

16. The anode of claim 10, wherein the or at least one of said electrochemically active constituent(s) is selected from the group consisting of oxides, oxyfluorides, phosphides, carbides and combinations thereof.

17. The anode of claim 16, wherein said oxides comprise spinels and/or perovskites.

18. The anode of claim 17, wherein said spinels are doped, non-stoichiometric and/or partially substituted spinels, the doped spinels comprising dopants selected from the group consisting of Ti⁴⁺, Zr⁴⁺, Sn⁴⁺, Fe⁴⁺, Hf⁴⁺, Mn⁴⁺, Fe³⁺, Ni³⁺, Co³⁺, Mn³⁺, Al³⁺, Cr³⁺, Fe²⁺, Ni²⁺, Co²⁺, Mg²⁺, Mn²⁺, Cu²⁺, Zn²⁺ and Li⁺.

19. The anode of claim 18, wherein said spinels comprise a ferrite and/or a chromite, in particular a ferrite selected from the group consisting of cobalt, manganese, molybdenum, nickel and zinc ferrite, and mixtures thereof, or a chromite selected from the group consisting of iron, cobalt, copper, manganese, beryllium, calcium, strontium, barium, magnesium, nickel and zinc chromite.

20. The anode of claim 16, wherein the or at least one of said electrochemically active constituent(s) comprises at least one Lanthanide as an oxide or an oxyfluoride, in particular cerium oxyfluoride, and mixtures thereof.

21. The anode of claim 10, wherein the or at least one of said electrochemically active constituent(s) comprises at least one metal selected from iron, chromium, copper and nickel, and oxides, mixtures and compounds thereof.

22. The anode of claim 10, wherein the passivatable metal substrate is coated on an electronically conductive core covered with an oxygen barrier layer.

23. The anode of claim 22, wherein the oxygen barrier layer comprises chromium oxide or black non-stoichiometric nickel oxide.

24. The anode of claim 22, wherein the oxygen barrier layer is covered with at least one protective layer consisting of copper or copper and at least one of nickel and cobalt, and/or oxides thereof to protect the oxygen barrier layer by inhibiting its dissolution into the electrolyte.

25. A cell for the production of aluminium by the electrolysis of alumina dissolved in a fluoride-containing electrolyte, in particular cryolite, having at least one non-carbon metal-based anode comprising an electrically conductive passivatable metal substrate and a conductive coating having an electrochemically active surface according to claim 10.

26. The cell of claim 25, comprising at least one aluminium-wettable cathode.

27. The cell of claim 26, which is in a drained configuration, comprising at least one drained cathode on which aluminium is produced and from which aluminium continuously drains.

28. The cell of claim 26, which is in a bipolar configuration and wherein the anodes form the anodic side of at least one bipolar electrode and/or a terminal anode.

29. The cell of claim 26, comprising means to circulate the electrolyte between the anodes and facing cathodes and/or means to facilitate dissolution of alumina in the electrolyte.

30. The cell of claim 26, wherein during operation the electrolyte is at a temperature of 750°C to 970°C.

31. Use of the anode of claim 10 for the production of aluminium in a cell for the electrowinning of aluminium by the electrolysis of alumina dissolved in a fluoride-containing electrolyte, wherein oxygen ions in the electrolyte are oxidised and released as molecular oxygen on the electrochemically active anode coating.

32. A method of producing aluminium in a cell as defined in claim 25, comprising oxidising oxygen ions on the electrochemically active anode coating of the or each anode and producing aluminium on a cathode.

## Patentansprüche

1. Verfahren zur Herstellung einer kohlenstofffreien, auf Metall basierenden Anode einer Zelle zur elektrolytischen Gewinnung von Aluminium, insbesondere durch Elektrolyse von Aluminiumoxid, das in Fluorid enthaltendem Elektrolyten gelöst ist, wobei das Verfahren Beschichten eines Substrats aus elektrisch leitfähigem Metall, das gegen hohe Temperatur beständig ist, wodurch die Oberfläche davon passiv und im Wesentlichen inert gegenüber dem Elektrolyten wird, mit mindestens einer Schicht eines elektrochemisch aktiven Beschichtungsvorläufers in Form einer Aufschlämmung oder Suspension, die mindestens einen elektrochemisch aktiven Bestandteil oder eine Vorläufer desselben umfasst, und Wärmebehandlung der oder jeder Schicht auf dem Substrat, um eine Beschichtung zu erhalten, die an dem passivierbaren Metallsubstrat haftet, wodurch die Oberfläche der Anode elektrochemisch aktiv für die Oxidation von Sauerstoffionen gemacht wird, die an der Elektrolytgrenzfläche vorhanden sind.

2. Verfahren nach Anspruch 1, bei dem das passivierbare Metallsubstrat mindestens ein Metall ausgewählt aus Nickel, Kobalt, Chrom, Molybdän, Tantal und der Lanthanidenreihe, und deren Legierungen oder intermetallischen Verbindungen umfasst.

3. Verfahren nach Anspruch 1, bei dem die Beschichtung gebildet wird, indem ferner ein bindendes Material aufgebracht wird, das im Wesentlichen in Bezug auf Kryolith beständig ist, um die Bestandteile der Beschichtung zusammenzubinden und auf das passivierbare Metallsubstrat zu binden.

4. Verfahren nach Anspruch 1, bei dem die Beschichtung aus einer Aufschlämmung oder Suspension erhalten wird, die kolloidales oder polymeres Material enthält, insbesondere mindestens eines von Aluminiumoxid, Ceroxid, Lithiumoxid, Magnesiumoxid, Siliciumdioxid, Thoriumoxid, Yttriumoxid, Zirkoniumdioxid, Zinnoxid und Zinkoxid, und Kolloiden, die wirksame Bestandteile der Beschichtung oder Vorläufer derselben enthalten, alle in Form von Kolloiden oder Polymeren.

5. Verfahren nach Anspruch 1, bei dem Bestandteile des Beschichtungsvorläufers mit sich selbst umgesetzt werden, um die Beschichtung zu bilden, oder mindestens ein Bestandteil des Beschichtungsvorläufers mit dem passivierbaren Metallsubstrat umgesetzt wird, um die Beschichtung zu bilden.

6. Verfahren nach Anspruch 1, bei dem der Beschichtungsvorläufer auf das Substrat durch Walzen, Bürsten oder Sprühung aufgebracht wird.

7. Verfahren nach Anspruch 1, bei dem das passivierbare Metallsubstrat auf einen elektronisch leitfähigen Kern beschichtet wird und eine Sauerstoffsperrschicht auf dem Kern insbesondere durch Oxidation der Oberfläche des Kerns unter Bildung der Sauerstoffsperrschicht gebildet wird oder durch Aufbringen eines Vorläufers der Sauerstoffsperrschicht auf den Kern und Wärmebehandlung.

8. Verfahren nach Anspruch 7, bei dem die Sauerstoffsperrschicht mit mindestens einer Schutzschicht bedeckt wird, die aus Kupfer oder Kupfer und mindestens einem von Nickel und Kobalt besteht, und/oder Oxiden derselben, um die Sauerstoffsperrschicht zu schützen, indem ihre Auflösung in den Elektrolyten inhibiert wird.

9. Verfahren nach Anspruch 1 zur Rekonditionierung einer kohlenstofffreien, auf Metall basierenden Anode mit einem passivierbaren Substrat mit einer elektrochemisch aktiven Beschichtung, wenn mindestens ein Teil der aktiven Beschichtung inaktiv oder abgenutzt geworden ist, wobei das Verfahren die Befreiung der Oberfläche des Substrats vor der erneuten Beschichtung der Oberfläche mit einer Beschichtung umfasst, die aus der Aufschlämmung oder Suspension aufgebracht wird.

10. Kohlenstofffreie, auf Metall basierende Anode einer Zelle für die elektrolytische Gewinnung von Aluminium, insbesondere durch Elektrolyse von Aluminiumoxid, das in einem geschmolzenes Fluorid enthaltenden Elektrolyten gelöst ist, die ein elektrisch leitfähiges Metallsubstrat, das gegen hohe Temperatur beständig ist, wobei die Oberfläche davon passiv und im Wesentlichen inert gegenüber dem Elektrolyten wird, und eine elektrochemisch aktive Beschichtung umfasst, die an der Oberfläche des Metallsubstrats haftet, wodurch die Oberfläche der Anode leitfähig und elektrochemisch aktiv für die Oxidation von Sauerstoffionen, die an der Elektrolytgrenzfläche vorhanden sind, gemacht und gehalten wird, wobei die Beschichtung elektrochemisch aktive Bestandteile in einem Kolloid enthält, die aus mindestens einem elektrochemisch aktiven Bestandteil oder einem Vorläufer desselben in einer Kolloid enthaltenden Aufschlämmung oder Suspension erhältlich sind.

11. Anode nach Anspruch 10, bei der das passivierbare Metallsubstrat mindestens ein Metall ausgewählt aus Nickel, Kobalt, Chrom, Molybdän, Tantal und der Lanthanidenreihe und deren Legierungen oder intermetallischen Verbindungen umfasst.

12. Anode nach Anspruch 11, bei der das passivierbare Metallsubstrat Nickel-beschichtetes Kupfer ist.

13. Anode nach Anspruch 10, bei der die Beschichtung ferner mindestens einen Elektrokatalysator oder einen Vorläufer desselben zur Bildung von Sauerstoffgas umfasst, insbesondere Elektrokatalysator(en) ausgewählt aus Iridium, Palladium, Platin, Rhodium, Ruthenium, Silicium, Zinn und Zink, der Lanthanidenreihe und Mischmetall, und deren Oxiden, Mischungen und Verbindungen derselben.

14. Anode nach Anspruch 10, bei der die Beschichtung ferner ein bindendes Material umfasst, das im Wesentlichen gegenüber Kryolith beständig ist, zur Bindung der Bestandteile der Beschichtung aneinander und auf das passivierbare Metallsubstrat.

15. Anode nach Anspruch 10, bei der die Beschichtung eine wärmebehandelte Aufschlämmung oder Suspension ist, die mindestens ein wärmebehandeltes Kolloid oder Polymer ausgewählt aus wärmebehandeltem kolloidalem oder polymerem Aluminiumoxid, Ceroxid, Lithiumoxid, Magnesiumoxid, Siliciumdioxid, Thoriumoxid, Yttriumoxid, Zirkoniumdioxid, Zinnoxid und Zinkoxid, und Kolloiden, die aktive Bestandteile der Beschichtung oder Vorläufer derselben, alle in Form von wärmebehandelten Kolloiden oder Polymeren, enthält.

16. Anode nach Anspruch 10, bei der der oder mindestens einer der elektrochemisch aktiven Bestandteile ausgewählt ist aus der Gruppe bestehend aus Oxiden, Oxyfluoriden, Phosphiden, Carbiden und Kombinationen derselben.

17. Anode nach Anspruch 16, bei der die Oxide Spinelle und/oder Perovskite umfassen.

18. Anode nach Anspruch 17, bei der die Spinelle dotierte, nicht-stöchiometrische und/oder partiell substituierte Spinelle sind, wobei die dotierten Spinelle Dotiermittel ausgewählt aus der Gruppe bestehend aus Ti⁴⁺, Zr⁴⁺, Sn⁴⁺, Fe⁴⁺, Hf⁴⁺, Mn⁴⁺, Fe³⁺, Ni³⁺, Co³⁺, Mn³⁺, Al³⁺, Cr³⁺, Fe²⁺, Ni²⁺, Co²⁺, Mg²⁺, Mn²⁺, Cu²⁺, Zn²⁺ und Li⁺ umfassen.

19. Anode nach Anspruch 18, bei der die Spinelle ein Ferrit und/oder ein Chromit, insbesondere ein Ferrit ausgewählt aus der Gruppe bestehend aus Kobalt-, Mangan-, Molybdän-, Nickel- und Zinkferrit und Mischungen derselben oder ein Chromit ausgewählt aus der Gruppe bestehend aus Eisen-, Kobalt-, Kupfer-, Mangan-, Beryllium-, Calcium-, Strontium-, Barium-, Magnesium-, Nickel- und Zinkchromit umfassen.

20. Anode nach Anspruch 16, bei der der oder mindestens einer der elektrochemisch aktiven Bestandteile mindestens ein Lanthanid als Oxid oder Oxyfluorid insbesondere Ceroxyfluorid und Mischungen derselben umfassen.

21. Anode nach Anspruch 10, bei der der oder mindestens einer der elektrochemische aktiven Bestandteile mindestens ein Metall ausgewählt aus Eisen, Chrom, Kupfer und Nickel und Oxide, Mischungen und Verbindungen derselben umfassen.

22. Anode nach Anspruch 10, bei der das passivierbare Metallsubstrat auf einen elektronisch leitfähigen Kern beschichtet ist, der mit einer Sauerstoffsperrschicht bedeckt ist.

23. Anode nach Anspruch 22, bei der die Sauerstoffsperrschicht Chromoxid oder schwarzes nicht-stöchiometrisches Nickeloxid umfasst.

24. Anode nach Anspruch 22, bei der die Sauerstoffsperrschicht mit mindestens einer Schutzschicht bedeckt ist, die aus Kupfer oder Kupfer und mindestens einem von Nickel und Kobalt besteht, und/oder Oxiden derselben, um die Sauerstoffsperrschicht durch Inhibierung ihrer Auflösung in den Elektrolyten zu schützen.

25. Zelle zur Herstellung von Aluminium durch Elektrolyse von Aluminiumoxid, das in Fluorid enthaltendem Elektrolyten gelöst ist, insbesondere Kryolith, mit mindestens einer kohlenstofffreien, auf Metall basierenden Anode, die ein elektrisch leitfähiges passivierbares Metallsubstrat und eine leitfähige Beschichtung mit einer elektrochemisch aktiven Oberfläche gemäß Anspruch 10 aufweist.

26. Zelle nach Anspruch 25, die mindestens eine mit Aluminium benetzbare Kathode umfasst.

27. Zelle nach Anspruch 26, die in einer mit Drainage versehenen Konfiguration vorliegt, die mindestens eine drainierte Kathode umfasst, in der Aluminium erzeugt wird und von der Aluminium kontinuierlich abläuft.

28. Zelle nach Anspruch 26, die in einer bipolaren Konfiguration vorliegt, und bei der die Anoden die anodische Seite mindestens einer bipolaren Elektrode und/oder eine terminale Anode bilden.

29. Zelle nach Anspruch 26, die Mittel zur Zirkulation des Elektrolyten zwischen den Anoden und gegenüberliegenden Kathoden und/oder Mittel zur Vereinfachung der Auflösung von Aluminiumoxid in dem Elektrolyten umfasst.

30. Zelle nach Anspruch 26, bei der während des Betriebs der Elektrolyt bei einer Temperatur von 750 °C bis 970 °C vorliegt.

31. Verwendung der Anode gemäß Anspruch 10 zur Herstellung von Aluminium in einer Zelle zur elektrolytischen Gewinnung von Aluminium durch Elektrolyse von Aluminiumoxid, das in Fluorid enthaltendem Elektrolyten gelöst ist, wobei Sauerstoffionen in dem Elektrolyten oxidiert und als molekularer Sauerstoff an der elektrochemisch aktiven Anodenbeschichtung freigesetzt werden.

32. Verfahren zur Herstellung von Aluminium in einer Zelle gemäß Anspruch 25, bei dem Sauerstoffionen an der elektrochemisch aktiven Anodenbeschichtung der oder jede Anode oxidiert werden und Aluminium an einer Kathode erzeugt wird.

## Revendications

1. Procédé de fabrication d'une anode métallique exempte de carbone d'une cuve pour l'électro-obtention d'aluminium, en particulier par l'électrolyse d'alumine dissoute dans un électrolyte contenant du fluorure, ledit procédé consistant à enrober un substrat de métal électriquement conducteur résistant à haute température et dont la surface devient passive et sensiblement inerte vis-à-vis de l'électrolyte, avec au moins une couche d'un précurseur de revêtement électrochimiquement actif sous la forme d'un coulis ou d'une suspension contenant au moins un constituant électrochimiquement actif ou un précurseur de celui-ci, et à traiter thermiquement la ou chaque couche sur le substrat pour obtenir un revêtement adhérent au substrat métallique pouvant être passivé rendant la surface de l'anode électrochimiquement active pour l'oxydation d'ions oxygène présents au niveau de l'interface de l'électrolyte.

2. Procédé selon la revendication 1, dans lequel le substrat métallique pouvant être passivé comprend au moins un métal choisi à partir de nickel, colbalt, chrome, molybdène, tantale et la série des lanthanides, et leurs alliages ou composés intermétalliques.

3. Procédé selon la revendication 1, dans lequel le revêtement est formé en appliquant de plus une matière de liaison sensiblement résistante à la cryolite pour lier ensemble les constituants du revêtement et sur le substrat métallique passivable.

4. Procédé selon la revendication 1, dans lequel le revêtement est obtenu à partir d'un coulis ou d'une suspension contenant une matière colloïdale ou polymère, en particulier au moins une parmi l'alumine, l'oxyde de cérium, la lithine, la magnésie, la silice, la thorine, l'yttria, la zircone, l'oxyde d'étain et l'oxyde de zinc, et des colloïdes contenant des constituants actifs du revêtement ou des précurseurs de celui-ci, tous sous la forme de colloïdes ou de polymères.

5. Procédé selon la revendication 1, consistant à faire réagir des constituants du précurseur de revêtement entre eux pour former le revêtement, ou à faire réagir au moins un constituant du précurseur de revêtement avec le substrat métallique pouvant être passivé pour former le revêtement.

6. Procédé selon la revendication 1, dans lequel le précurseur de revêtement est appliqué sur le substrat par des rouleaux, à la brosse ou par pulvérisation.

7. Procédé selon la revendication 1, consistant à enrober le substrat métallique passivable sur un noyau électroniquement conducteur, et à former une couche d'arrêt à l'oxygène sur le noyau en particulier en oxydant la surface du noyau pour former la couche d'arrêt à l'oxygène, ou en appliquant un précurseur de la couche d'arrêt à l'oxygène sur le noyau et à traiter thermiquement.

8. Procédé selon la revendication 7, consistant à recouvrir la couche d'arrêt à l'oxygène avec au moins une couche protectrice composée de cuivre ou de cuivre et d'au moins l'un de nickel et de colbalt, et/ou des oxydes de ceux-ci pour protéger la couche d'arrêt à l'oxygène en inhibant sa dissolution dans l'électrolyte.

9. Procédé selon la revendication 1, pour remettre en état une anode à base de métal exempte de carbone ayant un substrat pouvant être passivé avec un revêtement électrochimiquement actif, quand au moins une partie du revêtement actif est devenu non actif ou usé, ledit procédé consistant à clarifier la surface du substrat avant d'enrober à nouveau ladite surface avec un revêtement appliqué à partir dudit coulis ou de ladite suspension.

10. Anode à base de métal exempte de carbone d'une cuve pour l'électro-obtention d'aluminium, en particulier par l'électrolyse d'alumine dissoute dans un électrolyte contenant du fluorure, comprenant un substrat métallique électriquement conducteur résistant à haute température, dont la surface devient passive et sensiblement inerte vis-à-vis de l'électrolyte, et un revêtement électrochimiquement actif adhérent à la surface du substrat métallique réalisant et conservant la surface de l'anode conductrice et électrochimiquement active pour l'oxydation d'ions oxygène présents au niveau de l'interface de l'électrolyte, ledit revêtement contenant des constituants électrochimiquement actifs dans un colloïde pouvant être obtenu à partir d'au moins un constituant électrochimiquement actif ou d'un précurseur de celui-ci dans un coulis ou suspension contenant le colloïde.

11. Anode selon la revendication 10, dans laquelle le substrat métallique pouvant être passivé comprend au moins un métal choisi à partir de nickel, cobalt, chrome, molybdène, tantale et la série des lanthanides, et leurs alliages ou composés intermétalliques.

12. Anode selon la revendication 11, dans laquelle le substrat métallique pouvant être passivé est du cuivre plaqué de nickel.

13. Anode selon la revendication 10, dans laquelle le revêtement comprend de plus au moins un électrocatalyseur ou un précurseur de celui-ci pour la formation de gaz oxygène, en particulier un (des) électrocatalyseur(s) choisi(s) à partir d'iridium, de palladium, de platine, de rhodium, de ruthénium, de silicium, d'étain et de zinc, de la série des lanthanides et de mischmétal, et leurs oxydes, mélanges et composés de ceux-ci.

14. Anode selon la revendication 10, dans laquelle le revêtement comprend de plus une matière de liaison résistant sensiblement à la cryolite pour lier ensemble les constituants du revêtement et sur le substrat métallique pouvant être passivé.

15. Anode selon la revendication 10, dans laquelle le revêtement est un coulis ou une suspension thermiquement traité contenant au moins un colloïde ou un polymère traité thermiquement choisi à partir d'alumine, d'oxyde de cérium, de lithine, de magnésie, de silice, de thorine, d'yttria, de zircone, d'oxyde d'étain et d'oxyde de zinc colloïdaux ou polymères traités thermiquement, et de colloïdes contenant des constituants actifs du revêtement ou des précurseurs de ceux-ci, tous sous la forme de colloïdes ou de polymères traités thermiquement.

16. Anode selon la revendication 10, dans laquelle le ou au moins l'un desdits constituants électrochimiquement actifs est choisi à partir du groupe composé d'oxydes, d'oxyfluorures, de phosphures, de carbures et de combinaisons de ceux-ci.

17. Anode selon la revendication 16, dans laquelle lesdits oxydes comprennent des spinelles et/ou des perovskites.

18. Anode selon la revendication 17, dans laquelle lesdits spinelles sont des spinelles dopés, non-stoïchiométriques et/ou partiellement substitués, les spinelles dopés contenant des dopants choisis à partir du groupe composé de Ti⁴⁺, Zr⁴⁺, Sn⁴⁺, Fe⁴⁺, Hf⁴⁺, Mn⁴⁺, Fe³⁺, Ni³⁺, Co³⁺, Mn³⁺, Al³⁺, Cr³⁺, Fe²⁺, Ni²⁺, Co²⁺, Mg²⁺, Mn²⁺, Cu²⁺, Zn²⁺ et Li⁺.

19. Anode selon la revendication 18, dans laquelle lesdits spinelles comprennent une ferrite et/ou une chromite, en particulier une ferrite choisie à partir du groupe composé de ferrite de cobalt, manganèse, molybdène, nickel et zinc, et de mélanges de celles-ci, ou une chromite choisie à partir du groupe composé de chromite de fer, cobalt, cuivre, manganèse, béryllium, calcium, strontium, baryum, magnésium, nickel et zinc.

20. Anode selon la revendication 16, dans laquelle le ou au moins l'un desdits constituants électrochimiquement actifs comprend au moins un lanthanide comme oxyde ou oxyfluorure, en particulier un oxyfluorure de cérium, et ses mélanges.

21. Anode selon la revendication 10, dans laquelle le ou au moins l'un desdits constituants électrochimiquement actifs comprend au moins un métal choisi à partir de fer, chrome, cuivre et nickel, et ses oxydes, mélanges et composés.

22. Anode selon la revendication 10, dans laquelle le substrat métallique pouvant être passivé est enrobé sur un noyau électroniquement conducteur recouvert d'une couche d'arrêt à l'oxygène.

23. Anode selon la revendication 22, dans laquelle la couche d'arrêt à l'oxygène comprend de l'oxyde de chrome ou un oxyde de nickel non stoïchiométrique noir.

24. Anode selon la revendication 22, dans laquelle la couche d'arrêt à l'oxygène est recouverte d'au moins une couche protectrice composée de cuivre ou de cuivre et d'au moins l'un de nickel et de cobalt, et/ou leurs oxydes pour protéger la couche d'arrêt à l'oxygène en inhibant sa dissolution dans l'électrolyte.

25. Cuve pour la production d'aluminium par l'électrolyse d'alumine dissoute dans un électrolyte contenant du fluorure, en particulier de la cryolite, ayant au moins une anode à base de métal exempte de carbone comprenant un substrat métallique pouvant être passivé électriquement conducteur et un revêtement conducteur ayant une surface électrochimiquement active selon la revendication 10.

26. Cuve selon la revendication 25, comprenant au moins une cathode mouillable par l'aluminium.

27. Cuve selon la revendication 26, qui est dans une configuration de drainage, comprenant au moins une cathode de drainage sur laquelle de l'aluminium est produit et à partir de laquelle l'aluminium s'écoule de façon continue.

28. Cuve selon la revendication 26, qui est dans une configuration bipolaire et dans laquelle les anodes forment le côté anodique d'au moins une électrode bipolaire et/ou une anode terminale.

29. Cuve selon la revendication 26, comprenant des moyens pour faire circuler l'électrolyte entre les anodes et les cathodes en vis-à-vis et/ou des moyens pour faciliter la dissolution de l'alumine dans l'électrolyte.

30. Cuve selon la revendication 26, dans laquelle, pendant le fonctionnement, l'électrolyte est à une température de 750°C à 970°C.

31. Utilisation de l'anode de la revendication 10 pour la production d'aluminium dans une cuve pour l'électro-obtention d'aluminium par l'électrolyse d'alumine dissoute dans un électrolyte contenant du fluorure, où des ions oxygène dans l'électrolyte sont oxydés et libérés comme oxygène moléculaire sur le revêtement anodique électrochimiquement actif.

32. Procédé pour produire de l'aluminium dans une cuve telle que définie dans la revendication 26, consistant à oxyder des ions oxygène sur le revêtement anodique électrochimiquement actif de l'anode ou de chaque anode et à produire de l'aluminium sur une cathode.
